

## UNITED STATES PATENT OFFICE

CHARLES T. HENNIG, OF CLEVELAND, OHIO

## PURIFICATION OF STEEL IN THE BESSEMER PROCESS

No Drawing.

Application filed August 16, 1929. Serial No. 386,490.

This invention relates to the manufacture of steel and more especially to the Bessemer process, whether acid or basic.

In the Bessemer process, as heretofore conducted, the resultant steel has not been entirely satisfactory, for many purposes, because of the fact that it carried a relatively large amount of iron oxide, manganese oxide and other impurities. Bessemer steel, as heretofore manufactured, has also been relatively high in nitrogen. These impurities have rendered Bessemer steel unsuitable for many uses, such as sheets for drawing purposes, certain grades of wire, and rails. In the steel trade, Bessemer steel, as heretofore made, has been commonly designated as a "dirty" steel because of the above mentioned impurities.

The inclusion of oxides, in Bessemer steels as heretofore manufactured, has been the result of the action of the oxygen in the air used for the "blow" combining with the metal elements of the molten mass, since the air is disseminated throughout the molten mass and the oxygen contacts with practically every particle thereof. For these reasons the manufacture of steel by the Bessemer process has been on the decline in this country for many years and its use has been restricted to certain products, such as pipes, bolts and other products requiring a free-cutting stock.

Another factor that has accelerated the decline in the Bessemer process in this country has been the development of the open-hearth process because of the possibility of using a greater variety of materials in the open-hearth process than in the Bessemer process.

It is one of the objects of the present invention to improve the Bessemer process so as to enable the production of cleaner steel or, in other words, steel having a lower content of dissolved oxides therein, which permits the use of such steel for a greater variety of products, because of its greater ductility.

It is a further object of the invention to improve the Bessemer process so as to enable the manufacture thereby of steels that are, generally speaking, equal to corresponding steels made by the open-hearth process and I have found that, in some instances, it is possible to make steels by my improved Bessemer process that are superior to corresponding steels made by the open-hearth process.

The Bessemer process has many commercial advantages over the open-hearth process and among these advantages are the fact that the steel can be made in a few minutes by the Bessemer process whereas it takes many hours by the open-hearth process and that the process is more flexible in that many grades or analyses of steel may be made from the amount of metal that would be necessary for a heat in an open-hearth furnace and, in the case of an open-hearth furnace, all of the metal of each heat would necessarily conform to a single specified analysis. In other words, the metal that would be used to make a one hundred ton heat in an open-hearth furnace, all of which would be of one kind of steel to meet one specification, could by the Bessemer process be made into any number of different kinds of steel depending upon the size of converter used.

It is common practice to use from two to twenty-five tons of molten metal in a "blow", depending upon the equipment of the plant and the demand for the steel.

In carrying out my invention, the molten metal from the blast furnace, cupola or mixer, is charged into the converter in the usual way and the "blow" is made in the usual way and, upon the completion of the "blow", the metal is poured into the pouring ladle. After a small amount of the metal has been poured into the pouring ladle, I throw into the ladle a charge of purifying material, such as is disclosed in my earlier application No. 301,434, filed August 22, 1928 and which consists es-

sentially of a mixture of commercial soda ash and a controlling substance therefor, such as manganese dioxide. The purifier, in addition to the materials specified, contains some lime 5 to raise the melting point of the soda ash, and may vary as to its composition but I have found that the following composition is entirely satisfactory:

|                                                                             | Per cent |
|-----------------------------------------------------------------------------|----------|
| 10 Commercial soda ash ( $Na_2CO_3$ )                                       | 80       |
| Calcium oxide ( $CaO$ ) as limestone                                        | 2 to 6   |
| Manganese dioxide ( $MnO_2$ )                                               | 1/4 to 1 |
| Chlorine, as calcium chloride ( $CaCl_2$ )<br>or sodium chloride ( $NaCl$ ) | 1/2      |

15 The balance consists of a binder and impurities in the form of silica, magnesia, iron and alumina. The materials, in the proportions specified, are made up in the form of 20 briquets and the binder that is used in these briquets is preferably glucose or molasses refuse, which is mixed with the other materials of the briquets, in a heated condition, and then run through a machine in which the mixture 25 is pressed into briquet form. These briquets are preferably of a size that would weigh about three ounces each.

The amount of briquets to be used varies 30 with the quality of steel desired and may run from one-half to three pounds per ton of metal. The briquets are usually put into a paper bag and this bag is thrown into the ladle while the metal is being poured into it from the converter and should be put in prior 35 to the time that the manganese is added, because the purifier tends to protect the manganese against oxidation and, therefore, permits of the use of a smaller amount of manganese than has heretofore been the practice. 40 The addition of the purifier results in an immediate and energetic ebullition of the metal which carries the included gases and impurities to the top where the impurities are held by the slag and the gases pass out 45 through the slag and are entirely eliminated. The action of the purifier lasts for about a minute and then the metal is thoroughly degasified and cleansed of the oxides and other impurities which it originally contained. 50 The resultant slag is liquid and very quiet and acts as a seal for the surface of the metal and the fact that the slag is quiet indicates that the metal has been thoroughly degasified. The metal is then ready for pouring into the molds. 55

If the metal is over-oxidized in the "blow" and has a tendency to not lie quietly in the first mold, some of the purifier may be added to each of the other molds, either on the stool 60 or during the pouring, and this will result in the metal lying quietly in the molds. For this purpose, about one-fourth of an ounce to one ounce per ton of metal should be added to each mold.

65 If the metal from the blast furnace, cupola

or mixer is not in the right condition because of the presence of an excessive amount of oxides and other impurities, this condition can be corrected by the use of some of the purifier either in the transfer ladle or converter, or 70 both, and from one-half pound to one pound and a half may be used for this purpose, depending upon the appearance of the metal, it being understood that those skilled in the art are able to detect the condition referred to 75 from the appearance of the metal and by such appearance will be able to determine the amount of the purifier that is to be used in any case. When the purifier is put into the transfer ladle, it acts on the metal in the 80 ladle and the metal with the slag containing the purifier is then poured into the converter where the purifier continues its action. In some cases the purifier may also be put into the converter where the condition of the metal 85 is unusually bad or, if preferred, in some cases, the purifier may be put in the converter and not in the transfer ladle. When the purifier is put into the converter, it is preferable to do this either before the metal is run in or 90 before the "blow" starts.

Having thus described my invention, what I claim is:

1. The herein-described method of purifying steel in the Bessemer process of manufacture which consists in treating the molten metal, after it has been blown, with a deoxidizing material in the form of an intimate mixture comprising commercial soda ash and manganese dioxide and wherein the soda ash 100 is over three-fourths of the mixture and the manganese dioxide is an effective amount, up to five per cent, for controlling the action of the soda ash as and for the purpose described.

2. The herein-described method of purifying steel in the Bessemer process of manufacture which consists in treating the molten metal, after it has been blown, with a deoxidizing material in the form of an intimate mixture comprising commercial soda ash, a calcium compound and manganese dioxide and wherein the soda ash is over three-fourths of the mixture, the calcium compound has a calcium oxide content that is an effective amount, up to ten per cent, to substantially 110 raise the melting point of the soda ash, and the manganese dioxide is an effective amount, up to five per cent, for controlling the action of the soda ash as and for the purpose described.

3. The herein-described method of purifying steel in the Bessemer process of manufacture which consists in treating the molten metal, after it has been blown, with lumps of a deoxidizing material in the form of an intimate mixture comprising commercial soda ash, a calcium compound, and manganese dioxide, and wherein the soda ash is over three-fourths of the mixture, the calcium compound has a calcium oxide content that is an effec- 120 125 130

tive amount, up to ten per cent, to substantially raise the melting point of the soda ash, and the manganese dioxide is an effective amount, up to five per cent, for controlling the action of the soda ash as and for the purpose described.

In testimony whereof, I hereunto affix my signature.

CHARLES T. HENNIG.

10

15

20

25

30

35

40

45

50

55

60